

March 15, 1960

H. B. WHITEHURST ET AL

2,928,716

METHOD OF PRODUCING GLASS FIBERS WITH METAL COATINGS

Filed Nov. 5, 1952

2 Sheets-Sheet 1



FIG. 1.



FIG. 2.

INVENTORS:  
HARRY B. WHITEHURST &  
WILLIAM H. OTTO

BY  
*Stackin & Germain*  
ATTORNEYS

March 15, 1960

H. B. WHITEHURST ET AL

2,928,716

METHOD OF PRODUCING GLASS FIBERS WITH METAL COATINGS

Filed Nov. 5, 1952

2 Sheets-Sheet 2

FIG. 3.



INVENTORS:

HARRY B. WHITEHURST &  
WILLIAM H. OTTO

BY  
*Steckin & Oberman*  
ATTORNEYS

FIG. 4.

2,928,716

## METHOD OF PRODUCING GLASS FIBERS WITH METAL COATINGS

Harry B. Whitehurst, Granville, and William H. Otto, Newark, Ohio, assignors to Owens-Corning Fiberglas Corporation, a corporation of Delaware

Application November 5, 1952, Serial No. 318,786

9 Claims. (Cl. 18—54)

This invention relates to glass fibers and particularly to fibers treated to provide strands, yarns, and other textiles having increased abrasion resistance and knot strength. In particular, it relates to coating glass fibers with metals and metal alloys in a way to enhance the properties of the fibers.

It is an object of the invention to apply a metal coating to glass fibers to protect the surfaces and to apply the coating in such a way as to enhance other properties of the fibers.

It is another object of the invention to coat the fibers at temperatures that assure uniform coatings on the fibers and that secure good tensile strength and other properties of the fibers.

In more detail, it is an object to control the temperature of the glass as it is being drawn and as it passes from a molten state to a solidified state with reference to the molten metal to be applied so that the thermal history of the glass fiber is adapted to impart the best properties to the finished product.

In the drawings:

Figure 1 is a schematic side elevational view of apparatus for producing glass fiber strands;

Figure 2 is a front elevational view of the same apparatus;

Figure 3 is a central longitudinal sectional view on the line 3—3 of Figure 2 depicting the relationship of parts on a greatly enlarged scale; and

Figure 4 is a front elevational view of a part of the present invention.

Attempts have been made to provide glass fibers with a metal coating which completely surrounds each individual fiber and thereby protects it from adjacent fibers in a strand. The purpose was to increase the abrasion resistance of the fibers to such a point that strands, yarns, and fabrics made from such fibers have greatly increased resistance to abrasion, flexing, knotting, and other working which in the case of previously produced glass fiber textiles often was destructive. We have found that the properties of the metal-coated glass fibers, especially the uniformity and effectiveness of coating, the abrasion and flexure resistance, and the tensile strength, were bettered by attention to the thermal experience of the glass strand as it flows from its source, is drawn out into fibers, and is coated with molten metal.

In accordance with the present invention, the molten metal is applied to the fiber or stream immediately after the stream has been drawn out into a fiber and at a point where the stream is at substantially the same temperature as the molten metal being applied to the stream. In this way, the metal coating apparently forms on the glass fiber under ideal conditions. In addition, the thermal experience of the glass fiber itself is apparently adapted to impart to the finished product the best possible properties.

Metals that may be applied according to the present invention include most of the common low temperature melting metals, such as Wood's alloy, Rose's metal, lead,

alloys of lead and tin, lead and zinc, tin and zinc, brass, bronze, and others. For example, an alloy composed of 99% zinc and 1% titanium may be applied to the fibers at temperatures of about 800° F. Other metals and alloys and their preferable temperatures of application are:

|                                                             | ° F. |
|-------------------------------------------------------------|------|
| Zinc                                                        | 840  |
| Tin                                                         | 750  |
| 10 90% tin, 10% silver                                      | 570  |
| Alloy 151B (a predominantly tin-silver alloy)               | 800  |
| Alloy Cerroseal 35 (approximately half tin and half indium) | 250  |

15 Referring to the drawings, Figure 1 depicts in schematic fashion a fiber producing apparatus which includes a receptacle and feeder 10 for molten glass that may be heated in any conventional manner. The feeder 10 is provided with a series of outlets 12 in its bottom, from 20 which flow a plurality of streams 14 of molten glass. Preferably, the outlets are all arranged in one or two rows so that the streams as they flow from the outlets are all substantially in the same plane. As the streams flow from the outlets 12 they are drawn out into fibers 25 16 by means of a rotating drum 18 which winds the fibers thereon, and through the winding action exerts a pulling force on the fibers to draw out the streams. Intermediate the source of the streams of molten glass and the winding drum 18 a guide shoe 20 is provided with a groove 30 to collect the fibers into a group or strand 22, in which relation the fibers are wound on the drum 18. Various coating and sizing materials may be applied to the fibers as they are being grouped into the strand, for example, a binding material such as starch or synthetic resin may 35 be run onto the shoe to coat the fibers and the strand and secure the fibers together in the strand. The coating or sizing material may also contain a lubricant for the metal-coated fibers, such as petroleum oil, vegetable oil, molybdenum disulfide, wax or other recognized lubricants for metal.

The means for applying molten metal to the fibers as they are being formed includes an applicator 24 which, as shown in Figures 2 and 4, is an elongated receptacle made of graphite and of substantially L shape having a 45 narrow trough 26 extending substantially the full length thereof and enclosed within the vertical extending part of the L-shaped container. The horizontally extending part of the L-shaped container ends in a face 28 which has a plurality of slots 29 therein and through which the fibers 50 14 pass as they are attenuated on their way to being grouped into a strand. Each one of the slots 29 is connected by means of a small passage 32 with the trough 26 so that molten metal in the trough 26 feeds through the passages to the slots 29. By proper regulation of the 55 level of the molten metal in the trough 26, which can be accomplished by control of the rate of feed of the metal into the trough, sufficient head is maintained on the metal in the passage 32 to force it as a small drop into the slot 29 where, due to its surface tension, it seeks to 60 remain and resist displacement by the glass fiber 14 being drawn through the slot. The glass fiber passing through the slot becomes completely encased in the drop of metal in the slot so that it is coated with a layer of metal which completely surrounds the fiber and extends uniformly and substantially continuously and uninterruptedly over the fiber surface.

65 The metal in the applicator is maintained in molten state by heating the applicator by suitable means. For instance, the body of the applicator may be wound with an electric resistance element 25 which in turn is covered with a layer of insulation 30 such as sillimanite. The

resistance element is connected across terminals 27 to which electrical connection is made.

Figure 3 illustrates one example of the present invention employing metals melting at temperatures in the neighborhood of 700° F.

This view shows the stream 12 of molten glass flowing from the orifice in the feeder and being drawn out into a fiber 14. The fiber passes through the slot 29 in the end of the applicator 24 and passes through the glob of molten metal in the slot at the end of the passage 32.

The molten glass is indicated as being at a temperature of 2200° F., which is an approximate average of the temperatures employed for most glasses that are manufactured into textile fiber form.

It is presumed that shortly after the molten glass flows from the orifice in the feeder, the temperature of the glass drops to approximately 2000° F. as shown in Figure 3 and then through the drawing-out or attenuating range the glass temperature drops quickly to a value considerably below that at the feeder outlet. At a distance of two or three inches below the end of the opening in the feeder, the stream or fiber will have dropped to about 700° F. If the molten metal is at a temperature of 700° F. then the applicator for the molten metal is located at the point where the stream would normally be at 700° F. so that the stream and the molten metal are at the same temperature.

If desired, the applicator may be at a point where the stream temperature would be slightly above this point, say about 725° F., to assure that when the molten metal is applied to the stream the temperature of the stream will be substantially equal to the temperature of the molten metal but not lower than the molten metal temperature. Metal temperatures of 5° F. to 25° F. below glass temperature are usually sufficient. In this way there is no reheating of the stream so that any possible adverse effect upon the properties of the glass is avoided.

Shortly after the point at which the molten metal is applied to the stream, the coated stream or fiber falls quickly to room temperature and the fiber together with other similarly coated fibers is wound into a package on the drum 18.

To obtain the metal application to the fibers while the glass and metal are at the same temperature, the applicator is positioned sufficiently close to the outlet in the feeder to assure that the glass will not have time to cool below the temperature of the metal. However, if space requirements limit the approach of the applicator to the feeder, or if the metal being applied is one that is molten only at such high temperature that it would require that the applicator be placed closer to the feeder than is practicable, it may be desirable to incorporate in the glass composition some ingredient which will darken the color of the glass and thereby slow down radiation of heat from the interior of the glass stream to prolong the time during which the glass of the stream is at high temperature to thereby afford a greater space between the feeder and the applicator.

For instance, copper and other coloring agents may be added to the glass to darken the color of the glass and aid it in retaining its heat for a longer period of time. An example of a glass containing copper and which would operate in this way is as follows:

|                                | Percent |
|--------------------------------|---------|
| SiO <sub>2</sub>               | 55.90   |
| Al <sub>2</sub> O <sub>3</sub> | 5.50    |
| MgO                            | 2.55    |
| CaO                            | 6.05    |
| BaO <sub>3</sub>               | 4.50    |
| Na <sub>2</sub> O              | 2.60    |
| K <sub>2</sub> O               | 0.20    |
| SiO                            | 11.30   |
| CuO                            | 9.60    |
| Li <sub>2</sub> O              | 1.80    |

In place of copper oxide, other oxides such as lead, vanadium, or other oxides ordinarily used in the glass industry for darkening the color of glass, may be added to the glass compositions conventionally used for the manufacture of fibers.

Various modifications may be made in the invention within the spirit and scope of the appended claims.

We claim:

1. In the method of making glass fibers which comprises flowing a stream of molten glass from a supply thereof, drawing out the stream to a fiber and cooling the stream as it is drawn out to solidify it in the form of a fiber, the step of forming a coating of metal on the fiber by applying molten metal to the glass stream at a place along the stream where the glass of the stream is at a temperature substantially the same as the temperature of the molten metal immediately prior to its application to the stream.

2. In the method of making glass fibers which comprises flowing a stream of molten glass from a supply thereof, drawing out the stream and cooling the stream as it is drawn out to solidify it in the form of a fiber, the step of forming a coating of metal on the fiber by passing the stream through a body of molten metal so located along the stream that the stream as it engages the body of metal is at a temperature substantially the same as the temperature of the molten metal and solidifying on the fiber surface the metal so applied.

3. In the method of making glass fibers in which a stream of molten glass is flowed from a supply thereof, the stream is drawn out and cooled as it is drawn out to solidify it into a fiber, the step of forming a coating of metal on the fiber by passing the stream through a body of molten metal so located along the stream, that the stream as it engages the body of metal is at a temperature 5 to 25° F. above the temperature of the molten metal.

4. The method of making glass fibers which comprises continuously flowing streams of molten glass from a supply thereof, continuously drawing out the streams and cooling the streams as they are drawn out to solidify them in the form of fibers, forming coatings of metal on at least some of the individual fibers by passing at least some of the streams through bodies of molten metal so located along the stream that the streams as they engage the bodies of metal are at a temperature substantially the same as the temperature of the molten metal, and solidifying on the fibers the metal so applied.

5. The method of making glass fibers which comprises continuously flowing streams of molten glass from a supply thereof, continuously drawing out the streams and cooling the streams as they are drawn out to solidify them in the form of fibers, continuously collecting the drawn-out streams into a strand, forming a coating of metal on the individual fibers by applying to the streams before they are collected into the strand a molten metal that is applied to the streams at such a place along the streams that the temperature of the glass is substantially the same as the temperature of the molten metal prior to its application, and solidifying on the fiber surfaces the metal so applied.

6. The method of making glass fibers which comprises flowing streams of molten glass from a supply thereof, drawing out the streams and cooling the streams as they are drawn out to solidify them in the form of fibers, collecting the drawn-out streams into a group to form a strand, coating the streams before they are collected into the group with a molten metal that is applied at a point along the streams where the temperature of the glass is substantially the same as the temperature of the metal prior to its application, solidifying the metal coating, and applying a second coating material to the streams as they are collected into the group.

7. The method of making glass fibers which comprises flowing a stream of molten glass from a supply thereof, drawing out the stream and cooling the stream as it is

drawn out to solidify it in the form of a fiber, and passing the stream through a body of molten metal located at a point where the glass of the stream is at a temperature 5 to 25° F. above the temperature of the molten metal prior to its application.

8. The method of making glass fibers which comprises continuously flowing streams of molten glass from a supply thereof, continuously drawing out the streams and cooling the streams as they are drawn out to solidify them in the form of fibers. Continuously collecting the drawn-out streams into a group to form a strand, and applying to the streams before they are collected into the group a molten metal that is applied at a place where the temperature of the glass of the stream is 5 to 25° F. above the temperature of the molten metal prior to its application.

9. The method of making glass fibers which comprises continuously flowing streams of molten glass from a supply thereof, continuously drawing out the streams and cooling the streams as they are drawn out to solidify them

10

15  
20

in the form of fibers, continuously collecting the drawn-out streams into a group to form a strand, and passing the streams through bodies of molten metal individual to the streams before collecting the streams into a group,

5 the bodies of metal being so located along the streams that the glass of the streams comes into engagement with the metal before the glass has cooled to a temperature below the temperature of the molten metal.

References Cited in the file of this patent

UNITED STATES PATENTS

|           |         |               |
|-----------|---------|---------------|
| 2,053,923 | Stewart | Sept. 8, 1936 |
| 2,224,149 | Fisher  | Dec. 10, 1940 |
| 2,272,588 | Simison | Feb. 10, 1942 |
| 2,373,078 | Kleist  | Apr. 3, 1945  |
| 2,616,165 | Brennan | Nov. 4, 1952  |

FOREIGN PATENTS

|         |        |               |
|---------|--------|---------------|
| 840,209 | France | Jan. 11, 1939 |
|---------|--------|---------------|